

Dec. 31, 1935.

H. W. NIEMAN

2,025,768

APPARATUS FOR AND METHOD OF APPLYING TIN TO METALLIC SHEETS

Filed Aug. 15, 1931

2 Sheets-Sheet 1



Inventor

Henry W. Nieman

By R. S. C. Dougherty

Attorney

Dec. 31, 1935.

H. W. NIEMAN

**2,025,768**

# APPARATUS FOR AND METHOD OF APPLYING TIN TO METALLIC SHEETS

Filed Aug. 15, 1931

2 Sheets-Sheet 2



Inventor

Henry St. Nieman,

884 R. S. C. Wougherty, Attorney

## UNITED STATES PATENT OFFICE

2,025,768

APPARATUS FOR AND METHOD OF APPLY-  
ING TIN TO METALLIC SHEETSHenry W. Nieman, Bethlehem, Pa., assignor to  
Bethlehem Steel Company, a corporation of  
Pennsylvania

Application August 15, 1931, Serial No. 557,406

11 Claims. (Cl. 91—70.2)

This invention relates to methods of and apparatus for applying tin coatings to the surfaces of metallic sheet strips or the like.

Various types of machines are now employed 5 for the purpose of applying tin coatings to metallic sheets and are well-known in the metal working industry. Generally speaking, each such appliance includes a receptacle, known as a "tin pot", through which the sheet is passed, a bath of 10 molten tin being contained in the tin pot, and the sheet, in passing through this bath of molten tin, picking up a sufficient amount of the tin to adequately cover and coat its surfaces. It has been found difficult, however, to apply a perfect tin 15 coating in most instances, particularly where large quantities of metal, such as very long strips, are continually passed through the tin bath, as the molten tin becomes gradually contaminated with impurities known as particles of scruff or 20 "dead metal" which adhere to the sheet when it passes through the bath and which, when they pass through the tinning rolls, result in roughening or disfigurement of the surfaces.

Solid impurities which tend to collect in a 25 tin bath and to contaminate the same may be divided into three classes. The first class comprises light particles of carbon and dirt which settle through the palm oil, which is universally maintained above the surface of the tin, and rest 30 on the top surface of the body of molten tin. The second class includes particles, mainly iron, which amalgamate with the tin and settle down to the bottom of the tin pot. The third class comprises particles which partially amalgamate but, 35 owing to their small size, porosity, or admixture with lighter constituents, accumulate just below the top surface of the tin, forming a layer with an indefinite lower boundary.

The lighter particles, which settle downwardly 40 through the layer of palm oil, are easily prevented from reaching the surface of the tin by means of shields such as are well-known in the art. However, the light and heavy impurities in the tin bath are difficult to handle and have up until this 45 time constituted a serious obstacle in the tinning processes now in commercial use. Thus, these particles in the tin bath differ in specific gravity only slightly from that of the tin itself so that they tend to float around in the tin and, even 50 when they ultimately reach either the upper surface of the tin layer or fall to the bottom of the tin pot, are very easily dislodged by any current which may exist in the body of the molten tin and then carried into contact with the sheets 55 passing through the apparatus. Heretofore,

therefore, it has generally been considered essential to provide a relatively large tin bath and to avoid agitation of the bath. Even by taking such precautions, however, satisfactory results have not been realized, particles of heavy material in the portion of the bath directly above the strip contacting with the strip as they fall and the lighter particles below the strip tending to rise and foul the strip on coming in contact therewith.

In accordance with the present invention, I provide a definite circulation of the tin in the tin pot and also provide means for continuously cleaning the circulating tin and for causing the stream of molten tin thus cleaned to come in 10 contact with the metallic sheet passing through the tin pot. By the method just suggested and by suitable apparatus which will hereinafter be more fully described, it is possible to pass a metallic sheet through a tin pot without having 15 the sheet come in contact with any appreciable number of solid particles which tend to interfere with the perfection of the tinning process.

The invention is not limited in its broader aspects to any particular type of apparatus, and 20 the method may be carried out in tin pots which vary widely in design and arrangement of their component elements. That form of apparatus which is illustrated in the accompanying drawings is set forth by way of example only. The 25 method of and means for cleansing the tin may also be used quite independently of the actual tinning operation.

In the drawings:

Figure 1 shows, in longitudinal section, a tin 30 pot which is generally of a type now in common use but in which certain changes have been made in order to facilitate carrying out the improved process;

Figure 2 is an end view of the tin pot, partially 35 broken away to show the interior, and also showing in elevation, affixed thereto, the tin cleaning apparatus; and

Figure 3 is an axial section through the tin 40 cleaning apparatus.

The tin pot is indicated generally at 10 and is seen to comprise a portion 10' adapted to contain a part of the bath of molten tin (indicated at 11) and a small body of molten flux (indicated at 12), the portion 10' being in communication with the portion 10<sup>2</sup> of the pot only through an elongated arcuate passageway 13 defined by the curved shields 14, 14. The portion 10' of the tin pot contains a portion of the tin 45 bath, the level of the upper surface of which 50

bath is indicated at 15, and also a relatively deep body of palm oil, the level of the upper surface of which body is indicated at 16. Guide rolls arranged in pairs are indicated at 17, by means of which the incoming sheet of metal, which is moving in the direction of the arrow A, is guided into the passage between the shields 14, and pairs of tinning rolls positioned in the palm oil bath are indicated at 18, these rolls engaging the sheet of metal after it has emerged from the tin bath and being intended to remove the surplus tin and to produce a thin uniform coating.

In the main, the arrangement of parts just described is well-known. In accordance with my invention, however, I provide transverse manifolds 20 horizontally disposed along the upper edges of the shields 14, each of these manifolds being provided with series of apertures 21 directed toward the sheet of metal 22 passing between them. In the operation of the apparatus, molten tin is caused to flow through the manifolds 20 under light pressure and to be delivered in a large number of small streams 25 through the apertures 21 against the surface of the metallic sheet. This tin has previously been purified by means hereinafter to be described, and the streams of tin, after impinging against the metallic sheet, join and flow downwardly 30 through the duct or neck between the shields 14, streams of clean tin therefore sweeping downwardly along the sheet 22 on both sides thereof and finally emerging into the main bath of tin in the portion 10' of the tin pot. Hence it is 35 clear that not only is the sheet of metal actually passing between the shields 14 in contact with pure, uncontaminated, molten tin but that this molten tin is flowing in streams directed oppositely to the direction of movement of the incoming metallic sheet, so that any impurities which may have come into contact with the sheet are washed off by the action of the flowing streams of tin. In this way impurities are prevented 40 from clinging to the sheet which, when it reaches the tinning rolls 18, has a coating of pure tin. The resulting product presents an improved and 45 practically perfect surface.

The means for purifying the tin will now be described. It will be noted in Figure 1 that 50 there is present in the portion 10' of the tin pot, and below the level of the surface of the tin, a tin off-take pipe 25. This pipe is also shown in Figures 2 and 3 and will be seen to lead to a point below the cylindrical casing 26 of the 55 purification apparatus and there turns upwardly, passing through a hollow trunnion 26' mounted in a frame member 27 and discharging into the bottom of a cylindrical drum 28. The drum 28 is mounted on trunnion 26' and hence 60 is revolvably mounted in the frame member 27, and at the top of the apparatus a second frame member 29 is provided through which a shaft 30 extends, this shaft having its upper end connected to a driving motor 31 and its lower end 65 fixed in a spider 32 which bridges the reduced neck 33 extending axially from the upper end of cylinder 28. Cylinder 28 is therefore freely revolvable and is supported by frame members 27 and 29 for free rotation by the electric motor 70 31. Midway of the top and bottom of the cylinder 28 is a horizontal partition 35, which partition is provided with a plurality of spaced relatively small apertures 36. Mounted upon the upper side of the partition and disposed coaxially with the cylinder 28 is a cylindrical block 75

37. The neck 33 terminates in an annular flange or lip 38 which extends laterally and in close proximity to an annular channel 39 surrounding the neck.

As may be seen from Figure 2 of the drawings, 5 the discharge end of the tin conduit 25 is positioned below the level of the upper surface of the tin bath in the compartment 10' of the tin pot, and hence there is a tendency for the tin to flow from the tin pot into the lower compartment 10 of the rotatable drum 28. An annular shield 40, secured to the upper end of conduit 25, causes the tin to flow outwardly and onto the bottom of cylinder 28 as it emerges from the end of pipe 25 and prevents it from finding its 15 way down between the cylindrical inner surface of trunnion 26 and the cylindrical outer surface of the pipe 25.

In the operation of the device, the cylinder 28 is rotated at relatively high speed, and the 20 tin flowing into the cylinder through pipe 25 is immediately thrown downwardly against the wall of the cylinder by centrifugal action. Ultimately a thick layer of tin is built up against this wall, and the inner surface of this tin layer 25 will occupy some such position as indicated at 30 42. Naturally a quantity of the tin immediately flows through apertures 36 into the upper compartment, and when a sufficiently thick layer is built up in this compartment, as indicated by 35 the line 43, tin will begin to pass into the neck 33 and, inasmuch as this neck flares upwardly, will rise rapidly in the neck and ultimately be discharged over the flange 38 and into the annular stationary trough 39, from which trough 35 it will pass by gravity into the pipe 44.

Pipe 44 is positioned above the manifolds 20 and is connected to the ends of these manifolds so that the tin will flow downwardly and into the manifolds, creating a pressure in the manifolds and causing the jets of tin to flow outwardly through orifice 21 and against the metal sheet 22 in the manner heretofore described. Due to centrifugal action, the particles or impurities which are lighter than the tin will be 45 collected in the first compartment of the cylinder 28, being thrown toward the center of this compartment so that they come to occupy positions in the inner layer of the body of tin contained in this compartment, such positions being indicated, for instance, at 46. These lighter impurities will be trapped in the lower compartment so long as the purifier remains in operation. The tin, still containing its heavier impurities, flows through the apertures 36 into the 55 upper compartment and will here be separated from such heavier impurities, which collect adjacent the wall of the cylinder, as for instance in a layer indicated at 47. The molten tin which ultimately flows upwardly through the neck 33 60 of the cylinder, has been separated from both its lighter and heavier impurities and is practically free from all impurities whatever. The partition 35 may be designated a baffle for preventing flow of the lighter impurities through the apparatus, 65 and the annular portion 28' of the top of the cylinder may be termed a baffle for blocking the passage of the heavier impurities.

In order that sufficient heat may be imparted to the apparatus to prevent freezing of the tin, 70 gas heating flames may be provided. For instance, a gas conduit 50 positioned below conduit 25 may be provided with a plurality of apertures 51, and the gas escaping through these apertures will provide heating flames 52 to main- 75

tain the tin flowing through conduit 25 sufficiently molten. Also the exterior surface of the cylinder 28 may be heated by gas flames 53 resulting from the combustion of gas issuing from apertures 54 in a gas manifold 55. To maintain a non-oxidizing or neutral atmosphere in the apparatus, particularly in the neck 33 and above the surface of the tin in trough 39, a neutral or reducing gas may be introduced into the apparatus above the upper level of the tin through a pipe 56. At 57 an overflow pipe is indicated, by means of which any excess quantity of tin flowing out from neck 33 may be returned to pipe 25. Normally the molten tin stands in this overflow pipe at the same level as the discharge end of conduit 25, with which it is in open communication.

The tin cleaning apparatus is maintained in operation as long as the process of tinning is carried on and is drained whenever the process is halted. It is simple in operation, having only one moving part, inexpensive to construct and operate, and efficient in operation. It will be observed that the centrifugal apparatus disclosed comprises not only a means for cleansing the tin as it flows through but also a pump, inasmuch as it withdraws molten tin from the tin pot at one level and returns it at a higher level. As a pump, the apparatus may have various uses other than in connection with a tin pot or process of tinning, particularly in the handling of molten metal, and its design may be considerably modified in adapting it to various uses.

Having thus described the invention, what is claimed as new and desired to be secured by Letters Patent is:—

1. The method of tinning by the use of a tin bath which comprises removing a portion of the molten tin from the bath, cleansing the same, and returning the cleansed tin to the bath in such manner that the surfaces of an object undergoing the tinning operation are swept by streams of the returning cleansed tin.

2. The method of tinning articles by the use of a tin bath which comprises continuously removing molten tin therefrom, cleansing the same, continuously returning the cleansed tin to the bath and simultaneously passing said articles through said bath.

3. The method of tinning comprising immersing an article to be tinned in a bath of relatively impure molten tin, removing said article from said bath and cleansing said article by a flow of relatively pure molten tin.

4. The method of tinning sheet material comprising passing said material through a tin bath, continuously removing molten tin from said bath, cleansing said tin and continuously returning the cleansed tin to the bath at points adjacent to the line of emergence of said sheet from said bath.

5. The method of tinning sheet material comprising immersing said material in a bath of relatively impure molten tin, removing said material from said bath, cleansing said material by a flow of relatively pure molten tin and passing said material through rollers maintained at a temperature above the melting point of tin.

6. Apparatus for tinning sheet material comprising a bath of molten tin, centrifugal means

for continuously cleansing molten tin, means for continuously transferring molten tin from said bath to said cleansing means and from said cleansing means to said bath, and handling means operative simultaneously with all of the above mentioned means for immersing in and removing said sheet material from said bath. 5

7. Apparatus for tinning sheet material comprising a bath of molten tin, rollers for introducing said sheet material into said bath, rollers disposed above said bath for removing said sheet material from said bath, elongated nozzle means disposed below said second mentioned rollers and directed against said sheet material, centrifugal means for removing heavy impurities from 15 molten tin, centrifugal means for removing light impurities from molten tin, pump means, conduit means connecting said bath with said pump means, and with said first and second mentioned centrifugal means, and conduit means connecting said centrifugal means with said nozzle means whereby a flow of molten tin from said bath is forced in succession through said centrifugal means and said nozzle means.

8. The process of coating a metal article with 25 a metal coating which comprises passing the article to be coated through a main bath of molten coating metal, discharging additional molten coating metal upon said article at a point above the point where said article leaves said main 30 bath, said metal being discharged in a continuous stream into said main bath and enveloping the article to be coated at the point where said article leaves said main bath, whereby contact of said article and the metallic oxide on the surface of said main bath is prevented.

9. The process of coating a metal article with a metal coating which comprises passing said article through a main bath of molten coating metal, discharging a continuous stream of like 40 coating metal upon said article at a point above the point where said article leaves said main bath, said metal being discharged in a continuous stream into said main bath and enveloping said article at the point where said article leaves 45 said main bath, whereby the metallic oxide on the surface of the bath is prevented from coming into contact with the article being coated.

10. The method of tinning comprising immersing articles to be tinned in a bath of relatively impure molten tin, continuously removing portions of said bath, purifying said portions and continuously circulating said purified portions over said articles. 50

11. The process of coating a metal article with 55 a metal coating which comprises passing said article through a main bath of molten coating metal, discharging a continuous stream of like coating metal upon said article at a point above the point where said article leaves said main 60 bath, said metal being discharged in a continuous stream into said main bath and enveloping said article at the point where said article leaves said main bath, whereby the metallic oxide on the surface of the bath is prevented from coming 65 into contact with the article being coated and maintaining a non-oxidizing environment about the point of discharge of said continuous stream into said main bath.